

## UNITED STATES PATENT OFFICE.

THOMAS DOW AINSLIE, OF METUCHEN, NEW JERSEY, AND RICHARD MARION LEVY, OF BROOKLYN, NEW YORK, ASSIGNORS TO THE ROESSLER & HASSLACHER CHEMICAL COMPANY, OF NEW YORK, N. Y., A CORPORATION OF NEW YORK.

## MANUFACTURE OF ARTICLES FROM WOVEN GOODS.

No Drawing.

Application filed July 19, 1923. Serial No. 652,655.

*To all whom it may concern:*

Be it known that we, THOMAS Dow AINSLIE and RICHARD MARION LEVY, citizens of the United States, and residents of Metuchen 5 and Brooklyn, in the counties of Middlesex and Kings and States of New Jersey and New York, respectively, have invented certain new and useful Improvements in the Manufacture of Articles from Woven Goods, 10 of which the following is a specification.

This invention relates to improved process for the manufacture of sewed articles from woven goods, and has particular reference to the manufacture of multi-ply or seamed 15 articles such as collars, cuffs, shirts, shirt bosoms, handkerchiefs, neck bands, under-wear, aprons, dresses, coats, trousers, vests, etc., from cotton, wool, linen, silk and other or mixed fibres.

20 The object of the invention is to effect a substantial saving in cost of manufacture under present methods, by the elimination of unnecessary handling operations, equipment, space, heat, and general overhead expense.

25 The invention is particularly applicable to large scale manufacture of soft, semi-soft, and stiff white collars, and as an example, without intending to limit ourselves thereby, we will describe the application of the in- 30 vention to large scale quantity manufacture of collars.

Prior to our invention the first step in the manufacture of white collars has been to 35 bleach, usually by chlorin, the gray or un-bleached piece goods-as it comes from the loom, the term "gray" being applied in the cotton piece goods trade to various colors ranging from yellow to dirty white or gray according to the variety of cotton employed.

40 The bleaching of such piece goods with chlorin requires a large space containing kiers, wash boxes, sour boxes, and bleaching machines, as well as drying cans, and tenter frames to bring the web properly to the 45 desired width. It also requires calenders and other finishing equipment. A large amount of heat and space are required for this boiling out, washing, souring, tentering, drying and calendering, drying and finishing 50 equipment, as well as considerable labor in handling. The dried piece goods then goes to the cutting room where it is dried out into

the blanks of the finish size, and the blanks are then assembled into the rough collar through the various operations of infolding, 55 sewing, buttonholing, etc. The rough collar may by this time have acquired considerable dirt and grease from the various machines and operations through which it has passed since the bleaching, and requires a 60 second bleaching and washing before the final laundering.

According to our invention, we cut over-size blanks from the unshrunk gray piece goods, assemble same into the rough un-bleached unshrunk and unlaundered collar, 65 then bleach same, wash and launder for use. By this method, we eliminate the objectionable bleaching room and equipment for handling piece goods, at least one drying 70 and one washing operation, and so materially simplify the manufacturing operations as to effect a saving of upwards of two cents per pound of finished goods.

We have discovered that the success of 75 the process is largely dependent upon the method of bleaching used because of the difficulty of reaching the inner plies without damaging the outside. If the bleaching is not complete, the inner gray along seams 80 creeps through in use and discolors the outside seams. We have obtained especially satisfactory results with a hydrogen peroxid bleaching method, to be more fully described hereinafter, although within the broad scope 85 of our invention we do not restrict ourselves to any particular kind of bleach other than one capable of complete penetration and effect without damaging the outside. A hydrogen peroxid bleaching process is suit- 90 able because of the release of nascent oxygen within the plies tending to produce a balloon effect and facilitating complete penetration.

It has heretofore been considered by those skilled in the large scale manufacture of 95 collars that the usual bleaches for piece goods either would not penetrate the several plies of the seams in a collar, or else would, before penetrating the inner plies, have weakened the outer plies, thereby damaging 100 the fabric and shortening its life. It has also been considered that it was impracticable to shrink a rough oversized collar to the desired standard size, and have it keep

to size and shape after repeated laundering, but in carrying out our invention on large scale production, we have overcome these objections with the resulting substantial 5 saving above stated.

The piece goods as it comes from the loom may be singed if desired, after which it is removed to the cutting room where the blanks are cut to larger size allowing for 10 shrinkage. For a 15 collar, the blanks will be cut between  $15\frac{1}{2}$  and  $15\frac{3}{4}$  size, preferably about  $15\frac{3}{4}$ , as it is preferable to have a finished collar slightly oversize than slightly undersize. Other sizes will be cut in proportion, including both the outside and the interlining where an interlining is used. This invention is applicable to soft and stiff collars made of separate neck band and outside sewed together, and also to semi-soft 15 collars which have recently come into the market made of one piece of special fabric and not intended to be starched. The blanks are preferably sewed together and button-holed with bleached thread, and the rough 20 unshrunk or oversize collar is then taken to the bleaching room and without any further treatment is immersed in the bleach liquor. If desired, cotton goods may be boiled out in an alkaline bath before bleaching, but the 25 bleaching is preferably done without boiling out or other prior treatment.

A suitable and preferably mildly alkaline bleach bath is 93% sodium peroxid from 2.5 to 6.0 lbs. per 100 lbs. of goods; or from 4 30 to 12 lbs. sodium peroxid per one hundred gallons of water. Approximately 1.3 lbs. of 66° Bé. sulphuric acid is used for each pound of sodium peroxid in order to partially neutralize the caustic soda resulting 35 from the reaction of sodium peroxid with water. As a retarding agent as well as an alkalining agent to permit proper penetration of the bleach to the interior plies, and at the same time to allow gradual liberation 40 of the nascent oxygen throughout the plies, about 5 lbs. of 42° Bé. sodium silicate is used for each 100 gallons of bleach liquor. The strength of the resulting hydrogen peroxid 45 bath ranges from  $\frac{1}{3}$  volume to 2 volumes, meaning that one gallon of bleach bath will 50 liberate from  $\frac{1}{3}$  to 2 gallons of active or nascent oxygen. The bleach is then washed out and the collar laundered and shrunk to size. A separate operation for shrinking 55 is not necessary, as shrinking occurs in the several foregoing operations.

The bleaching is best carried out at approximately 180° F. for 16 to 20 hours but can be from 120° to 212° according to the 60 material. For wool, 120° is suitable, and for boiled off silk, 145°, but for silk to be degummed and bleached in one bath, temperature up to boiling may be employed.

The practical advantages of this invention are that by bleaching the made up col-

lar, rather than the piece goods, there is a large saving in steam because of not having to dry the bleached collar before laundering. Also, the installation required for bleaching made up collars is less extensive 70 than that required for bleaching piece goods, because mangles, kiers, drying cans, tenter frames and calenders used in the former process prior to laundering are dispensed with. Also, there is a material saving in water required for washing before drying and cutting bleached piece goods. Labor and general overhead costs are materially less because of the reduction in the number of operations, handling, drying, cleaning, etc. 75 Also dirt acquired in the assembling and sewing is removed without special washing and a second bleaching, which latter tends to weaken the goods.

By the process herein described, all plies 80 of hems, seams, filling, etc. are completely bleached without reversion to gray even after prolonged exposure. Collars made by this process are of the desired size when dried after bleaching and remain so. Although we preferably only dried once after bleaching and laundering, which effects shrinkage to finish size, we do not restrict ourselves to drying and shrinking in laundering, but may dry and shrink to size after 85 bleaching without laundering. The sewing thread is preferably bleached, but either bleached or unbleached thread has no tendency to distort the assembled collar. The finished collar has a greater tendency to remain true to size and shape in subsequent 90 use than do collars made according to present methods and is more durable because of only being bleached once. As near as we can determine, the effectiveness of the bleach penetration throughout all plies is due to the liberation of the gas within the assembled collar between the plies which causes it to 95 swell up or balloon and thereby gives intimate contact of the active oxygen with all portions of the fabric. Other bleach baths capable of effecting the same result may be used within the broad scope of this invention.

In the appended claims the term "multiple layer," while applied to collars or other articles, includes not only those articles which have two or more layers of fabric throughout, but also those in which the finished article contains two or more substantially parallel layers of fabric in any component part such as are formed by hems, 100 seams, or bands.

We claim:

1. The process of manufacturing an article from woven fabric which consists in forming a rough oversized multiple layer article from unbleached piece goods, then bleaching and shrinking.
2. The process of manufacturing an article

- cle from woven fabric which consists in forming a rough oversized multiple layer article from unbleached piece goods, then bleaching and shrinking to a predetermined size.
3. The process of manufacturing an article from woven fabric which consists in forming a rough oversized multiple layer article from unbleached piece goods, bleaching in a bleach bath capable of releasing 10 bleaching gas throughout the layers, and shrinking.
4. The process of manufacturing an article from woven fabric which consists in forming a rough oversized multiple layer article from unbleached piece goods, bleaching in a bleach bath capable of releasing nascent oxygen throughout the layers, and shrinking to the predetermined size.
5. The process of manufacturing an article from woven fabric which consists in forming a rough oversized multiple layer article from unbleached piece goods, bleaching in a peroxid bleach, and shrinking to the predetermined size.
6. The process of manufacturing a collar or the like from woven fabric which consists in forming a rough oversized multiple layer collar from unbleached piece goods, then bleaching and shrinking.
7. The process of manufacturing a collar or the like from woven fabric which consists in forming a rough oversized multiple layer collar from unbleached piece goods, then bleaching and shrinking to the predetermined size.
8. The process of manufacturing a collar or the like from woven fabric which consists in forming a rough oversized multiple layer collar from unbleached piece goods, bleaching in a bleach bath capable of re-
- leasing bleaching gas throughout the layers, and shrinking.
9. The process of manufacturing a collar or the like from woven fabric which consists in forming a rough oversized multiple layer collar from unbleached piece goods, bleaching in a bleach bath capable of releasing nascent oxygen throughout the plies, and shrinking to the predetermined size. 45
10. The process of manufacturing a collar or the like from woven fabric which consists in forming a rough oversized multiple layer collar from unbleached piece goods, bleaching in a peroxid bleach at a temperature of upwards of 160° F., and shrinking to the predetermined size. 50
11. The process of manufacturing a collar or the like from woven fabric which consists in forming a rough oversized multiple layer collar from unbleached piece goods, sewing together with bleached thread, bleaching and shrinking to the predetermined size. 55
12. The process of manufacturing a collar or the like from woven fabric which consists in forming a rough oversized multiple layer article from unbleached piece goods, assembling and sewing same together, bleaching the assembled rough oversize collar throughout all layers and seams in an alkaline bath containing a retarding agent and a source of nascent oxygen at a temperature of approximately 180° F. without damaging the outer layers, and shrinking to the predetermined size. 60
- 70
- 75

Signed at Perth Amboy, in the county of Middlesex and State of New Jersey, this sixteenth day of July, A. D. 1923.

THOMAS DOW AINSLIE.  
RICHARD MARION LEVY